

# United States Patent Office

**2,951,040**

Patented Aug. 30, 1960

1

2,951,040

## **EXTREME PRESSURE LUBRICANTS CONTAINING MOLYBDIC XANTHATES**

**Georges Hugel, Ville d'Avray, Seine-et-Oise, and Robert Courtel, Paris, France, assignors to Institut Français du Pétrole des Carburants et Lubrifiants, Reuil-Malmaison, Seine-et-Oise, France**

No Drawing. Filed Jan. 7, 1955 Ser. No. 480,613

**Claims priority, application France Jan. 7, 1954**

6 Claims. (CL 252—336)

The present invention is concerned with lubricants containing molybdc xanthates and being capable of use under high temperature and pressure conditions.

It is known that the use of solid substances such as, for example, graphite or molybdenum sulfide, for coating the contact surface of metallic parts subjected to friction, facilitates the sliding thereof, considerably reducing their coefficient of friction and wear. Generally, this coating is realized with the aid of a solution prepared by incorporating into a lubricant (oil or grease) a colloidal suspension of graphite or of molybdenum sulfide. These thereupon form a deposit which fills the irregularities in the surfaces and protects them, even if the lubricant should happen not to reach any difficultly accessible parts of the contact surfaces. However, such a solution is bound up with the disadvantage which is inherent in every colloidal suspension, namely, that it is subject to flocculation under the influence of a change in the oil, which causes it to lose all its efficacy.

A primary object of the present invention is to remedy this deficiency. This is realized, briefly stated, by means of a solution prepared by dissolving in the oil or grease a soluble compound of molybdenum which decomposes under the influence of the temperatures and pressure locally attained by friction, said solution having the property of depositing a sulfur compound of molybdenum on the metallic surfaces.

Preferred, among the soluble compounds of molybdenum, are the molybdate xanthates of the formula



wherein R is an alkyl group since, according to the present invention, these decompose at the temperatures attained by friction.

Best adapted for good lubrication purposes are those xanthates of the preceding formula which are derivatives of higher alcohols. As a matter of fact, the solubility of these complexes in mineral oils increases with the length of the chain of the R radical. The solubility in oils is already very high when the R radical comprises 6 to 12 carbon atoms. The use of a long hydrocarbon chain affords still another advantage: it makes it possible to lower the temperature at which the molybdenum compound decomposes in the oil, e.g. from about 300° C. for the isobutyl derivative to about 170° C. for the decyl derivative.

Montequi (An. Espan. Fis. Quim. 1930, 28, 481) has described molybdc xanthates of the foregoing formula wherein the alkyl groups contain 2, 4 and 5 atoms, i.e. the ethyl, isobutyl and isoamyl derivatives. (Montequi did not envisage the possibility of using the said xanthates as lubricant additives.) The aforesaid molybdc xanthates wherein R contains from 6 to 12 carbon atoms

2

or more can be prepared in the manner set forth in the examples hereinafter set forth.

The solutions of molybdc xanthates in mineral oil can be used, according to this invention, to prepare an immersion bath for metallic parts whereby the latter can be covered with a tenaciously adherent brownish black coating of sulfur compound of molybdenum.

To obtain such a coating, the metallic part is immersed in a bath prepared by dissolving molybdic xanthate (preferably a derivative of a higher alcohol) in mineral oil, e.g. in an amount to provide a 0.5 to 10%, preferably an 8%, solution by weight, by heating the mixture to a temperature above the decomposition temperature of the molybdic xanthate (between about 170 and 15 380° C.) and maintaining such temperature for a period of from  $\frac{1}{2}$  hour to 2 hours.

Particularly good results are obtained at a temperature of about  $300^{\circ}$  to  $320^{\circ}$  C., maintained for a period of 2 hours. The duration of the treatment period can be reduced by employing a higher temperature.

The value of such a preliminary coating is clearly demonstrated by the result of tests carried out with the so-called "Four-Ball Machine" (as described by Boerlage in "Engineering," July 14, 1953, page 46). Using an oil which contains 2% by weight of molybdc decylxanthate: with a seizing delay of 2 seconds, pressures above 140 kg. could not be attained; with a seizing delay of 60 seconds, pressures above about 120 kg. could not be attained. On the other hand, if the balls were preliminarily provided with a coating as aforescribed, the pressure could be raised to about 310 kg. with a seizing delay of 15 seconds. This is a remarkable performance, the impression left on the balls not exceeding the plastic deformation due to these high pressures. There is thus practically no wear. The table which follows shows the principal results of tests carried out with an oil containing 2% by weight of molybdc decylxanthate:

### Results of tests on "Four-Ball Machine"

|    |                                                                             |     |     |      |                                          |     |     |     |      |     |
|----|-----------------------------------------------------------------------------|-----|-----|------|------------------------------------------|-----|-----|-----|------|-----|
| 40 | Oil S.A.E. 30+2% molybdc decylxanthate (Viscosity at 50° C.=54 centipoises) |     |     |      |                                          |     |     |     |      |     |
|    | Untreated balls                                                             |     |     |      | Balls subjected to preliminary treatment |     |     |     |      |     |
| 45 | Load applied (kg.)                                                          | 70  | 120 | 130  | 140                                      | 180 | 220 | 250 | 280  | 310 |
|    | Seizing delay (seconds.)                                                    | >60 | >60 | 18.3 | 0.8                                      | >60 | 55  | 43  | 26.5 | 15  |

It is evident from this table that the performances obtained when employing a preliminarily-applied protective coating are superior to those obtained with the aid of a lubricant alone.

55 However, this coating is subject to progressive elimination due to friction. To avoid such elimination, i.e. to retain the coating, it is preferred to use a lubricant containing in solution an organic compound of molybdenum which is decomposable under the influence of the 60 pressure and temperature produced by friction. Such a lubricant thus makes it possible constantly to renew the protective coating in proportion to its wear.

Illustrative of the lubricants suitable for this purpose are inter alia the following:

65 An oil containing in solution an organic compound of molybdenum, soluble in the oil and decomposable under the influence of the pressure and the temperature produced by friction, and particularly a mineral oil containing either a molybdic xanthate or hydrocarbon-soluble molybdenum blue.

A solution of a nitrogenous thiomolybdate in a vegetable or animal oil or in an oil constituted by a mixture of

esters of fatty acid and alcohol or by a mixture obtained from transesterification of vegetal or animal oils with polyethylene or polypropylene glycol or a higher alcohol, or by the synthetic products from the esterification of mono or polyalcohols with fatty acids or from the esterification of diacids with monoalcohols; and particularly a solution of a nitrogenous thiomolybdate in a diol, glycol, polyalcohol or polyethyleneglycol; the lubricants thus obtained having the property of decomposing at temperatures and pressures produced by friction.

Among others the following specific oils can be used as lubricants according to the invention:

Castor oil  
Peanut oil  
Olive oil  
Ox-foot oil  
Fish oil  
Monooleates of polyethylene glycols  
Monooleates of butylene glycols  
Monooleates of propylene glycols  
Monooleates of polytrimethylene glycols  
Palmitates of polypropylene glycols  
Dioleates of polyethylene glycols  
Dioleates of butylene glycol  
Dioleates of polypropylene glycols  
Dioleates of polytrimethylene glycols  
Bishexyl sebacate  
Bishexyl adipate  
Bishexyl methyl adipate  
Bisheptyl sebacate  
Bisheptyl adipate  
Bisheptyl methyl adipate  
Bisoctyl sebacate  
Bisoctyl adipate  
Bisoctyl methyl adipate  
Bisnonyl sebacate  
Bisnonyl adipate  
Bisnonyl methyl adipate  
Bisdecyl sebacate  
Bisdecyl adipate  
Bisdecyl methyl adipate  
Bisundecyl sebacate  
Bisundecyl adipate  
Bisundecyl methyl adipate  
Bisdodecyl sebacate  
Bisdodecyl adipate  
Bisdodecyl methyl adipate  
Decane diol  
Octane diol  
Hexane diol

Lubricants containing hydrocarbon-soluble molybdenum blue, as well as those obtained with the aid of a nitrogenous thiomolybdate, are disclosed and claimed in copending applications filed on even date herewith by Georges Hugel for "Hydrocarbon-Soluble Molybdenum Blues," Serial No. 480,612, filed January 7, 1955, now Patent No. 2,852,469 (corresponding to P.V. 661,055, filed in France on January 6, 1954) and for "Lubricants Containing Nitrogenous Thiomolybdates" (corresponding to P.V. 661,056, filed in France on January 6, 1954).

The present invention encompasses within the scope thereof lubricants produced with the aid of molybdc xanthates, and also those molybdc xanthates per se of the hereinbefore-given formula wherein R contains 6 or more carbon atoms, as for example molybdc decylxanthate, molybdc dodecylxanthate and molybdc hexylxanthate.

The principal results of tests using as lubricant, by way of example, an oil containing 2% by weight of molybdc decylxanthate, have been set forth above. The table which follows sets forth results obtained with the "4-Ball Machine," while insuring retention of the protective coating by means of an oil containing 1% by weight of molybdenum blue:

#### 4 Tests on "Four-Ball Machine"

##### OIL WITH 1% OF MOLYBDENUM BLUE

| 5                                                               | Load Applied in kg. | Delay in Seizing in seconds | Coefficient of Friction |                  |                                 | Diameter of Impression in mm. |
|-----------------------------------------------------------------|---------------------|-----------------------------|-------------------------|------------------|---------------------------------|-------------------------------|
|                                                                 |                     |                             | Before Seizing          | Maximum          | After Seizing                   |                               |
| BALLS SUBJECTED TO PRELIMINARY TREATMENT WITH MOLYBDIC XANTHATE |                     |                             |                         |                  |                                 |                               |
| 10                                                              | 280                 | >60                         | 0.14                    | extremely small. | coalescence of balls in 57 sec. | 0.82                          |
|                                                                 | 350                 | 39                          | 0.22                    |                  |                                 |                               |

15 This table shows that performances obtained while insuring retention of the protective coating by a lubricant with a hydrocarbon-soluble molybdenum blue base are remarkable since it is possible therewith to attain a pressure of 350 kg. with a seizing delay of 39 seconds.

20 It is also possible to use any one of the lubricants which come into consideration for the formation, and not only for the maintenance, of the said protective coating.

25 Comparable results are then attained provided that the increase in pressure is progressive and is effected with continuous lubrication. In fact, under the influence of the temperature attained by friction, a molybdenum sulfur compound is deposited in successive layers on metallic parts subject to friction, resulting simultaneously in the formation and in the maintenance of a protective coating.

30 The performances thus realized, with continuous lubrication by the progressive application of constantly increasing pressures, have already been set forth in connection with lubricants containing a nitrogenous thiomolybdate (thiomolybdate of an organic nitrogen base) in copending application, Ser. No. 480,611, filed January 7, 1955, now Patent No. 2,909,541 (corresponding to P.V. 661,056 in France). The table which follows sets forth results of tests obtained under the same conditions with a lubricant containing, for example, 2% by weight of molybdc decylxanthate:

##### Tests with "Four-Ball Machine"

45 [Mineral oil S.A.E. 30 (viscosity at 50° C.=54 centipoises) +2% by weight of molybdc decylxanthate (1 mm. at each load with the same balls, with progressively increasing pressures and without preliminary coating)]

| 50 | Load Applied in kg. | Delay in Seizing in seconds | Coefficient of Friction |         |               | Diameter of Impression in mm. |
|----|---------------------|-----------------------------|-------------------------|---------|---------------|-------------------------------|
|    |                     |                             | Before Seizing          | Maximum | After Seizing |                               |
| 55 | 130                 | >60                         | 0.09                    |         |               |                               |
|    | 150                 | >60                         | 0.14                    |         |               |                               |
|    | 180                 | >60                         | 0.16                    |         |               |                               |
|    | 200                 | >60                         | 0.13                    |         |               |                               |
|    | 240                 | >60                         | 0.25                    |         |               |                               |
|    | 260                 | >60                         | 0.23                    |         |               |                               |
|    | 280                 | >60                         | 0.24                    |         |               |                               |
|    | 300                 | >60                         | 0.18                    |         |               |                               |
|    | 320                 | >60                         | 0.18                    |         |               |                               |
|    | 340                 | >60                         | 0.15                    |         |               |                               |
| 60 | 380                 | >60                         | 0.11                    |         |               | 1.1                           |

65 The following examples set forth representative embodiments of preparing molybdc xanthates according to this invention (percentages are by weight and yields are molar yields):

##### Example 1

70 One mol of anhydrous ammonium molybdate (196 grams) is dissolved in a liter of water admixed with 10 kilograms of crushed ice in a container which is exteriorly cooled by ice.

75 A solution of 2 mols (512 grams) of sodium decylxanthate is prepared in 2.5 liters of water. This second solution is slowly added, while stirring vigorously, into the first-prepared ammonium molybdate solution. There is

produced a white precipitate which, on contact with the air, becomes rose-colored. After incorporation of all the xanthate and stirring for a half-hour, about two liters of acetic acid (diluted in a proportion of one volume of acetic acid for four volumes of water) are introduced dropwise, while cooling constantly, until a pH of 4 is attained. The obtained violet-red colored precipitate is then extracted with light petroleum ether.

The solution in petroleum ether, after decantation, is dried over anhydrous magnesium sulfate, filtered, and freed of petroleum ether by evaporation under reduced pressure on a water-bath. There are obtained as residue 400 grams of molybdc decylxanthate in the form of a very dark red, almost black, oily mass (which represents a yield of 70% relative to the theoretical yield). Molybdc decylxanthate corresponds to the formula:



This mass, which is very soluble in mineral oils, is preferably maintained under refrigeration until it is ready for use (by incorporation into a lubricant oil, according to the present invention).

*Example 2*

The process according to Example 1 is followed, except that the ammonium molybdate solution is intimately admixed with a solution in two liters of water of 2 mols (568 grams) of sodium dodecyloxanthate.

The procedure being otherwise the same, there are obtained 450 grams of molybdc dodecylxanthate, which represents a yield of 71% of the theoretical. Molybdc dodecylxanthate corresponds to the formula:



*Example 3*

Twenty parts by weight of ammonium molybdate are dissolved in 100 parts by volume of water. The resultant solution is poured into 1000 parts by weight of the solution in 250 parts by weight of water of 50 parts by weight of hexylxanthate.

Then there are gradually added 25 parts by volume of an aqueous acetic acid solution of 20% strength. The resultant organomolybdc compound is then extracted with benzene, the latter is eliminated from the extract by boiling on a water-bath, first under atmospheric pressure and finally under a pressure of 10 mm. of Hg. There are thus obtained 37 parts by weight of molybdc hexylxanthate, which corresponds to a yield of 76.4% of the theoretical. Molybdc hexylxanthate corresponds to the formula:



In the foregoing, parts by weight bear the same relation to parts by volume as do grams to milliliters.

In any of the foregoing examples the extraction of the molybdc xanthate may as well be achieved by means of a saturated paraffinic hydrocarbon having preferably less than 8 carbon atoms; such as for example pentane or isopentane, hexane-n, heptane-n, octane-n or mixtures such

- 5 pentane, hexane-n, heptane-n, octane-n or mixtures such as petroleum ether having a boiling point of 50 to 120° C.

According to the first of the aforementioned copending applications, a hydrocarbon-soluble molybdenum blue can

- be prepared from a molybdenum blue which is soluble e.g. 10 in isobutyl alcohol, by dissolving the last-mentioned blue in isobutyl alcohol to which has been added an organic liquid, such as a higher alcohol, which is simultaneously soluble in isobutyl alcohol and in hydrocarbons, then expelling the isobutyl alcohol, and finally concentrating the 15 remainder down to a suitable concentration whereby excess solvent is eliminated. The starting molybdenum blue can also be extracted from its aqueous solution by means of a phosphorus compound, such as diethylamido-di-decyl-phosphate, which is soluble in oil but not in water.

- 20 According to the second of the aforementioned co-pending applications, a thiomolybdate of an organic nitrogen base, as for example triethylamine, is prepared from a soluble thiomolybdate and a soluble salt, e.g. the hydrochloride of the base, whereby the desired organic  
25 base thiomolybdate is precipitated. These thiomolybdates are soluble in lubricant bases, including polyalcohols and the like, and are thermally decomposable to yield sulfur compounds of molybdenum for coating parts which are subject to friction.

- 30 Having thus disclosed the invention, what is claimed is:

  1. A lubricant consisting essentially of a mixture of about 90 to 99.5% by weight of a lubricating mineral oil and about 0.5 to 10% by weight of a molybdc xanthate having the formula



- 10 wherein R stands for an alkyl radical with 6 to 12 carbon atoms.

15 2. A lubricant according to claim 1 wherein the molyb-  
dic xanthate is molybdcic decylxanthate.

3. A lubricant according to claim 1 consisting essen-  
tially of about 98% by weight of the mineral oil and  
about 2% by weight of the molybdcic xanthate.

4. A lubricant according to claim 1 wherein the molyb-  
dic xanthate is molybdcic dodecylxanthate.

5. A lubricant according to claim 1 wherein the molyb-  
dic xanthate is molybdcic hexylxanthate.

6. A lubricant according to claim 1 consisting essen-  
tially of about 92% by weight of the mineral oil and  
about 8% by weight of the molybdcic xanthate.

**References Cited in the file of this patent**

UNITED STATES PATENTS

- |           |                 |                |
|-----------|-----------------|----------------|
| 1,740,809 | Cronshaw et al. | Dec. 24, 1929  |
| 2,173,383 | Carter          | Sept. 19, 1939 |
| 2,346,155 | Denison et al.  | Apr. 11, 1944  |
| 2,363,884 | McCleary et al. | Nov. 28, 1944  |
| 2,394,954 | Watkins         | Feb. 12, 1946  |
| 2,436,051 | Mixon           | Feb. 17, 1948  |
| 2,758,089 | Hoff et al.     | Aug. 7, 1956   |